

## UNITED STATES PATENT OFFICE

2,221,522

## FLOOR COVERING

Robert G. McLean, Chicago, Ill.

No Drawing. Application September 25, 1937,  
Serial No. 165,698

2 Claims. (Cl. 106—7)

The invention relates to improvements in floor coverings especially adapted for use as an indoor skating rink for ice skates and has for its primary object the provision of a compound of the character indicated by means of which an ordinary floor may be provided with a surface upon which ice skating may be done.

Another object of the invention is the provision of a covering of the character indicated upon which dancing may also be done.

Other objects will appear hereinafter.

The invention consists in the floor covering hereinafter described and claimed.

In making up the floor covering a mixture is first provided of ingredients as follows: hypo-sulphite of soda  $Na_2S_2O_5H_2O$ , 10 quarts; sodium borate, 42 ounces; sodium bicarbonate, 14 ounces; sodium fluoride  $NaF$ , 14 ounces, paraffine  $\frac{1}{2}$  pound.

These ingredients are mixed together and heated until they boil whereupon the mixture is poured upon the floor to be covered and allowed to solidify. The quantity of ingredients above specified will be found to be sufficient to cover thirty square feet of floor.

As will be noted, the bulk or base of the preparation consists of sodium hypo-sulphite and the function of the sodium borate, sodium bicarbonate, and sodium fluoride are to so harden the same as to adapt it to use with ice skates, the sodium borate and fluoride being particularly effective for this purpose. The paraffine wax tends to provide a smooth surface and when said surface is properly polished, in dancing or otherwise, will also serve as a suitable dancing surface or floor.

I have found that the hyposulfite of soda, the sodium bicarbonate and the paraffine are the most important ingredients and will of themselves provide a satisfactory floor covering, but that the addition of the other ingredients specified somewhat improve the consistency and skating qualities of the cover. I have also found that it is practically essential to include from 80% to 94% by weight of the hyposulfite, from 5% to 15% by weight of the sodium bicarbonate, and from 1% to 5% of the paraffine, depending upon the moisture content in the atmosphere in which the floor covering is to be used.

While I have set forth in detail the preferred ingredients and proportions, these are capable of some variation and modification without departing from the spirit of the invention. I therefore do not wish to be limited to the precise details disclosed, but desire to avail myself of such variations and modifications as fall within the scope of the appended claims.

I claim:

1. A floor covering composed of ingredients mixed together substantially in proportions as follows: hypo-sulphite of soda, 10 quarts; sodium borate, 42 ounces; sodium bicarbonate, 14 ounces; and sodium fluoride, 14 ounces.

2. A floor covering composed of ingredients mixed together substantially in proportions as follows: hypo-sulphite of soda, 10 quarts; sodium borate, 42 ounces; sodium bicarbonate, 14 ounces; sodium fluoride, 14 ounces; and paraffine wax,  $\frac{1}{2}$  pound.

ROBERT G. McLEAN. 35